

F. M. BECKET.

MANUFACTURE OF CALCIUM CARBID.

APPLICATION FILED APR. 10, 1916.

1,292,387.

Patented Jan. 21, 1919.



Witnesses  
G. T. Ball  
C. H. Potter

Inventor,  
Frederick M. Becket,  
Bynes, Transcend & Bruckmann,

Attorneys

# UNITED STATES PATENT OFFICE.

FREDERICK M. BECKET, OF NIAGARA FALLS, NEW YORK, ASSIGNOR TO UNION CARBIDE COMPANY, OF NEW YORK, N. Y., A CORPORATION OF VIRGINIA.

## MANUFACTURE OF CALCIUM CARBID.

1,292,387.

Specification of Letters Patent. Patented Jan. 21, 1919.

Application filed April 10, 1916. Serial No. 90,207.

To all whom it may concern:

Be it known that I, FREDERICK M. BECKET, a subject of the King of England, residing at Niagara Falls, in the county of Niagara and State of New York, have invented certain new and useful Improvements in the Manufacture of Calcium Carbid, of which the following is a specification.

This invention relates to the manufacture of calcium carbide, and particularly to improved processes for preparing a charge for reduction in the electric furnace. My present process involves a special procedure for preparing aggregates of the character described in my prior United States Patent No. 1,187,567, patented April 27, 1915.

According to said patent, aggregates suitable for furnacing are prepared by mixing lime with a suitable coking coal, in proper proportions as therein defined, and subjecting the mixture to heat under ordinary coking conditions. According to the present improvements aggregates of the desired character are prepared under special coking conditions which permit of a continuous or semi-continuous operation, whereby certain important advantages are secured, as hereinafter pointed out. As raw materials I employ a mixture of unburned limestone and a coking coal, or equivalent bituminous material, and I perform the operations of coking the coal and burning the limestone while conveying the charge through a heating zone, in which, preferably, the temperature increases toward the exit end. During the transit of the charge through the heating zone agitation or stirring of the mass is avoided.

My invention will be described in one specific illustrative embodiment, and in connection with apparatus as shown in the accompanying drawing, wherein the figure is a longitudinal central section. In said drawing—

1 represents a large heating chamber or tunnel-like structure of masonry, appropriately heat insulated. Within this chamber is mounted a conveying system for the charge, the essential characteristic of this system being that the mixture to be transformed into aggregates is maintained in a relatively quiescent state, that is to say, it is not subjected to material agitation or stir-

ring while it is being transported through the heating zone. As a diagrammatic illustration of one type of conveying systems conforming to this requirement, I have shown a continuous chain of relatively shallow cars or receptacles 2, which may be moved continuously or intermittently by any desired mechanism (not shown) in a direction preferably counter to that of the gases. These receptacles are filled successively from a storage bin 3 by means of any suitable mechanical feed device 4, and they discharge 65 their converted contents upon conveyer 5, by which the aggregates, after crushing if required, are carried to the carbid furnaces.

6 indicates a partition or apron extending from side to side of the tunnel, making a 70 tight joint with one end thereof, and depending at its forward end into proximity to the tops of the cars 2. 7 is a burner or equivalent means for supplying heat at a point or points adjacent the exit end of the tunnel. 75 If desired supplemental burners may be disposed at intervals along the walls as indicated by way of example at 8, 8. 9 is the outlet for the gases of combustion from the burners, commingled with carbon dioxide 80 derived from the limestone. The volatile products from the coking operation are largely withdrawn through the flue 10, and may be returned, preferably after being subjected to any usual treatment for the recovery of 85 valuable by-products including ammonia, to the burners 7, 8. Fuel from other sources, as for example coal, producer gas, oil or the like, is employed at the burners 7, 8, as may be required to supplement the heating effect 90 of the volatile products above mentioned.

A typical operation is as follows: Lime-stone is crushed, for example to grains having an average diameter of about one-eighth 95 inch more or less, and is intimately mixed with a highly bituminous coal crushed to a like or lesser size of particle. This mixture is fed from the storage bin 3 into the receptacles 2, partly or completely filling the 100 latter. The receptacles with their charge slowly traverse the heating zone. The time required for complete conversion will depend upon the temperature, and also upon the depth of the bed of mixture in the cars 105 2. With a depth of mixture not exceeding

six inches, and a temperature at the exit end of about 1100° C., a time of transit of about three to four hours will suffice for the production of aggregates of sufficient strength to endure the subsequent furnacing.

During the first stage of the heating the charge is moving beneath the apron 6 and is shielded from direct impingement of the flame; that is, the conditions to which the charge is subjected approximate more or less closely to those in a retort. The temperature of the charge is slowly raised and coking occurs, the bituminous constituents and volatile products from the coal passing through the flue 10 to the by-product plant, if such is provided. The apron 6 may extend so far, and the rate of movement of the cars may be so controlled, that most of the bituminous matter will be expelled by the time the receptacles emerge from under the protection of the apron.

From this point the charge is subjected to the direct influence of the flame, and the burning of the limestone to lime is accomplished, or at least completed. I have found that this operation does not involve the destruction or material weakening of the aggregates which have been formed during the preliminary heating stages. The fully converted charge is dumped onto the conveyor 5, and after breaking up is carried with as little loss of heat as is practicable to the carbid furnaces.

It has been found, in operating in this manner, that for the best results rather more fixed carbon is necessary than is theoretically required by the carbid-forming reaction—



This is in all probability due to the fact that some oxidation of carbon takes place by reaction with the carbon dioxide present in the furnace gases, according to the equation—



Accordingly, I prefer to provide about ten per cent. excess of fixed carbon in computing the charge. This may be provided by increasing the coking coal component of the mixture, or by adding a small proportion of coke or other form of carbon.

A typical charge for use in accordance with this invention may comprise a mixture of 100 parts by weight of unburned limestone with about 62 parts of a rich bituminous coal, represented for example by the analysis—

|    |                 |       |
|----|-----------------|-------|
| 60 | Volatile matter | 36.48 |
|    | Fixed carbon    | 57.93 |
|    | Ash             | 5.59  |

Due allowance must of course be made for the varying percentages of ash in the coal and of impurities in the limestone.

As compared with the production of aggregates by a coking process carried out in a by-product oven of ordinary type, the present process offers the following advantages, among others:—

(1) It becomes practicable to render the entire operation essentially continuous in character.

(2) The mixture to be transformed into aggregates may be heated in relatively shallow beds or masses instead of being heated in bulk through an inclosing wall. This not only affords a more efficient utilization of the heat, but a far more rapid coking is possible. For example such shallow masses as I have referred to above may be thoroughly converted during a transit period of three to four hours, as compared with sixteen to twenty hours required for the ordinary coking operation in a by-product oven of the usual type.

(3) These relatively small masses can be broken into fragments suitable for furnacing with much less production of fines.

(4) The small masses are in general more uniform in character than the bulk material from a by-product oven, there being in the present case little or no tendency to the local production of fines, which tendency is common in ovens of the by-product type.

(5) The present process affords a much better control of the temperature gradient during the coking operation, and this control has an important influence on the strength of the aggregates. For example, a too strong initial heating of the charge which tends always to the production of weak aggregates, is easily avoided by introducing a large proportion, or if necessary all, of the fuel at or near the exit end of the heating chamber. For the best results the charge should be heated relatively slowly at first, after which it may be brought rapidly to full temperature. This is very effectively accomplished in the present process by causing the charge to progress, either continuously or step by step, through a heating zone of which the temperature gradient rises toward the exit end. This effect is accentuated by the fact that the initial heating occurs practically under retorting conditions, as distinguished from heating by a direct flame.

(6) These small masses are readily and quickly cooled below the temperature of combustion of carbon in case it is desired to store the coked material. This is especially advantageous because the character of the product is such that it cannot be fully quenched with water, as is the practice in cooling the bulk material from an ordinary by-product coke oven.

The above enumerated advantages are possessed by the present process in common with the process disclosed and claimed in

my companion application Serial No. 90,206, filed herewith, according to which the limestone is burned to lime before being mixed with the coking coal, and is thereafter coked without stirring or agitation while being conveyed through the heating zone. In addition, the present process offers the great advantage that the coking operation and the burning of the limestone take place at different points in a single structure, whereby not only are the heat losses minimized, but the heat of the gases from the limestone burning operation is directly availed of for the coking; while on the other hand, the gases from the coking operation, either before or after the recovery of by-products, are available for the burning of the limestone, for which purpose they may be conveyed to the burners 7, 8, as diagrammatically indicated by the broken line in the figure. This interchange of heat in a single structure may, theoretically, obviate the necessity of supplying fuel from an extraneous source; and in practice the quantity of extra fuel will be small in proportion to that required when the burning of the limestone and the coking of the lime-coal mixture are carried out as independent operations.

Furthermore, according to the present process the limestone may be ground, before burning, to a much finer grain than it is practicable to employ in an ordinary lime-burning operation, either in an upright kiln or in the usual smooth-walled rotary kiln; and the liberation of the carbon dioxide from these finer particles occurs more readily.

While I preferably employ a coking coal of the type above described, or a mixture containing a sufficient proportion of such coal to assure the binding action, I may use other suitable carbonaceous materials: Thus in some cases the bituminous coal may be wholly or partly replaced by peat. The present invention is not restricted to the use of any particular carbonaceous material or mixture, provided the mixture thereof with the requisite proportion of unburned limestone is capable of yielding sufficiently strong aggregates by coking.

50 I claim:—

1. In the manufacture of calcium carbide, the process of preparing aggregates suitable for furnacing, which consists in mixing with unburned limestone a carbonaceous material serving as a source of carbon for the carbid-forming reaction and furnishing also a coking binder for the mass, and coking the resulting mixture and driving off carbon dioxide in transit through a heating zone, while avoiding stirring or agitation of the mass.

2. In the manufacture of calcium carbide, the process of preparing aggregates suitable for furnacing, which consists in mixing with unburned limestone a carbonaceous material

serving as a source of carbon for the carbid-forming reaction and furnishing also a coking binder for the mass, and coking the resulting mixture and driving off carbon dioxide in transit through a heating zone of increasing temperature, while avoiding stirring or agitation of the mass. 70

3. In the manufacture of calcium carbide, the process of preparing aggregates suitable for furnacing, which consists in mixing with unburned limestone a carbonaceous material serving as a source of carbon for the carbid-forming reaction and furnishing also a coking binder for the mass, the fixed carbon of the charge being somewhat in excess of the requirements of the carbid-forming reaction, and coking the resulting mixture and driving off carbon dioxide in transit through a heating zone, while avoiding stirring or agitation of the mass. 75

4. In the manufacture of calcium carbide, the process of preparing aggregates suitable for furnacing, which consists in mixing with unburned limestone a carbonaceous material serving as a source of carbon for the carbid-forming reaction and furnishing also a coking binder for the mass, the fixed carbon of the charge being somewhat in excess of the requirements of the carbid-forming reaction, and coking the resulting mixture and driving off carbon dioxide in transit through a heating zone of increasing temperature, while avoiding stirring or agitation of the mass. 90

5. In a process of preparing aggregates suitable for the production of calcium carbide, the step which consists in subjecting a mixture containing limestone and a suitable coking coal successively to a coking operation and a lime-burning operation while in transit through a heating zone. 100

6. In a process of preparing aggregates suitable for the production of calcium carbide, the step which consists in subjecting a mixture containing limestone and a suitable coking coal successively to a coking operation and a lime-burning operation, and separately withdrawing the gases from the coking operation. 110

7. In a process of preparing aggregates suitable for the production of calcium carbide, the step which consists in subjecting a mixture containing limestone and a suitable coking coal successively to a coking operation and a lime-burning operation while in transit through a heating zone, and separately withdrawing the gases from the coking operation. 115

8. In a process of preparing aggregates suitable for the production of calcium carbide, the steps which consist in subjecting a mixture containing limestone and a suitable coking coal successively to a coking operation and a lime-burning operation while in transit through a heating zone, and utilizing 125

the heated gases from the lime-burning operation for the preliminary coking of the mixture.

9. In a process of preparing aggregates suitable for the production of calcium carbide, the steps which consist in subjecting a mixture containing limestone and a suitable coking coal successively to a coking operation and a lime-burning operation while in transit through a heating zone, utilizing the heated gases from the lime-burning operation for the preliminary coking of the mixture, and utilizing the combustible gases from the coking operation for burning the limestone.

10. In a process of preparing aggregates suitable for the production of calcium carbide, the step which consists in conveying a charge containing limestone and a suitable coking coal through a coking zone while avoiding stirring or agitation thereof.

11. In a process of preparing aggregates suitable for the production of calcium carbide, the step which consists in conveying a charge containing limestone and a suitable coking coal through a coking zone while avoiding stirring or agitation thereof.

coking coal through a coking zone of increasing temperature while avoiding stirring or agitation thereof.

12. In a process of preparing aggregates suitable for the production of calcium carbide, the step which consists in conveying a charge containing limestone and a suitable coking coal, in the form of a relatively shallow bed or mass, through a coking zone, while avoiding stirring or agitation thereof.

13. In a process of preparing aggregates suitable for the production of calcium carbide, the step which consists in conveying a charge containing limestone and a suitable coking coal, in the form of a relatively shallow bed or mass, through a coking zone of increasing temperature, while avoiding stirring or agitation thereof.

In testimony wherof I affix my signature in presence of two witnesses.

FREDERICK M. BECKET.

Witnesses:

SIDNEY OTIS,  
MORY SCAFE.